

R. D. COOKE,  
MANUFACTURE OF ENAMELED WARE,  
APPLICATION FILED APR. 4, 1919.

1,316,018.

Patented Sept. 16, 1919.



Raymond D. Cooke INVENTOR

By  
Pennie Davis Marvin & Edmunds,  
ATTORNEYS

# UNITED STATES PATENT OFFICE.

RAYMOND DENNY COOKE, OF TERRE HAUTE, INDIANA, ASSIGNOR TO COLUMBIAN ENAMELING & STAMPING COMPANY, OF TERRE HAUTE, INDIANA, A CORPORATION OF INDIANA.

## MANUFACTURE OF ENAMELED WARE.

1,316,018.

Specification of Letters Patent. Patented Sept. 16, 1919.

Application filed April 4, 1919. Serial No. 287,650.

*To all whom it may concern:*

Be it known that I, RAYMOND DENNY COOKE, residing at 621 Poplar street, Terre Haute, in the county of Vigo, State of Indiana, have invented certain new and useful Improvements in the Manufacture of Enameled Ware; and I do hereby declare the following to be a full, clear, and exact description of the invention, such as will enable others skilled in the art to which it appertains to make and use the same.

This invention relates to the manufacture of enameled ware and more particularly to the production of enameled ware from sheet steel, or similar metal, and to the treatment of the sheet steel as a preliminary to the enameling operation.

In the production of enameled ware, the steel is customarily pickled in acid solutions to clean the surface and the enameling is then carried out as expeditiously as possible to guard against the oxidation of the clean surface; and it has been an axiom of the enameling industry that the presence of oxid on the surface of the steel was a condition to be strenuously guarded against.

The usual procedure followed in preparing the steel for enameling is briefly as follows: The steel is received in the form of rolled sheets and is pressed or drawn into the form of culinary or other utensils. To facilitate this drawing operation, and to permit the steel to pull freely through the dies, an emulsion of mineral oil is applied to the sheet.

After the utensil has been shaped the customary operation is the removal of the oil by scaling. The practice in this operation is to dip the ware in an acid bath and while wet with the acid to heat it to redness for several minutes. By this treatment the oil is burned off, and the coating of iron oxid which results is in a condition to be removed by the action of a pickling solution. Or the oil may be removed by scrubbing the utensil with a soap solution or soap powder or similar detergent. In either case it is necessary that the steel be subsequently cleaned by subjecting it to a pickling treatment, that is by immersing it for some time in an acid solution to remove the oxid. The acid solution is usually a solution of mineral acids, such as sulfuric or hydrochloric acids, or an acid-

containing solution such as a solution of sodium acid sulfate. 55

The operations thus commonly employed for the removal of the oil from the steel and for the cleaning of the steel are expensive, and the apparatus therefor occupies considerable space. If the oil is removed by heating, a furnace is necessary for the carrying out of the heating operation. The operation of scrubbing with a detergent is likewise an expensive operation. Where hot pickling liquids are employed, the provision of heating means is necessary. The pickling operation consumes considerable time, is of a disagreeable character, and requires considerable apparatus and space therefor, while the coat of acids and of steam for heating 60 forms a very considerable element of expense 65 in the operation of an enameling plant. 70

According to the present invention the preliminary treatment of the oiled surface of the sheet steel for the removal of oil, and the 75 subsequent pickling thereof prior to the enameling operation, are avoided, and the sheet steel with its oiled surface is subjected to a combined heating and oxidizing operation which leaves the surface of the sheet 80 steel in a condition well adapted for the enameling treatment.

The present invention is based upon the discovery that, contrary to what has been 85 commonly believed, freedom from oxid of the steel surface to be enameled is not necessary; that the usual operations of cleaning, pickling and washing can be avoided; that the oil or grease present on the steel after 90 the drawing operation can be removed, and the steel placed in condition for the enameling operation, by a simple regulated heating of the steel ware to the proper degree; and that the resulting steel ware, which has an 95 oxid coating, is well adapted for use, without further treatment, in the enameling operation.

As the result of my investigations, I have been led to believe that the formation of a 100 layer of oxid takes place, in the common enameling operation, while the steel with its enamel coating is being heated to the required temperature for the fusion of the enamel, and that the formation of such an oxid layer under the enamel is essential to 105 the proper adherence and smoothness of the

enamel; and I have found that the enameling operation can be promoted by the formation of a proper oxid coating upon the steel prior to the application of the enameling 5 composition thereto and the subsequent firing operation.

In the practice of the present invention, the steel ware with its coating of oil is subjected to a short heating operation at such 10 a temperature that the oil will be quickly volatilized or burned and the steel will be oxidized to the desired degree. It has been found that the amount of oxygen taken up by the steel, when thus oxidized, was about 15 0.0004 gram per square centimeter, or that the amount of iron oxid formed was about 0.0014 gram per square centimeter. The oxid formation should be such that the steel has a pronounced blue color. In general, the 20 steel should have as deep a blue color as possible, without becoming black. I have obtained good results in the practice of the invention, by carrying out the heating operation in a gas furnace maintained at a tem- 25 perature of about 700° C. and by subjecting the steel ware to the temperature of such a furnace for a period of about thirty seconds. In this time the steel being treated does not reach the temperature of the furnace, and 30 consequently the oxidation is not carried as far as when the steel itself becomes red hot. A different temperature or time of heating, which will produce the desired blue oxid coating, may be used in place of the particu- 35 lar conditions above mentioned.

A gas fired furnace of the leir type has been found well adapted to the practice of the invention. I have thus used to advantage a furnace having a fire brick tunnel 40 16 feet long, 30 inches wide and 12 inches high at the center, with the gas burners placed below the bottom of the furnace, and with circulation of the gases therefrom through openings between the bottom and 45 sides of the furnace. The burners were so arranged that all or any portion of the length of the furnace could be heated and were provided with an automatic constant temperature control. An endless chain was 50 run through the furnace over the sprockets at each end, so that the ware could be fed in at one end and taken out at the other. The speed of the chain and the length of the heated zone of the furnace were so adjusted 55 that the ware could be subjected to a temperature of about 700° C. for about thirty seconds. The time and temperature can, however, be somewhat varied to bring about the desired oxidation, *i. e.*, to produce a deep 60 blue color. By increasing the length of the furnace and correspondingly increasing the speed of the chain, the capacity of the furnace can be similarly increased.

A furnace of the character above referred 65 to is illustrated, in a conventional and dia-

grammatic manner, in the accompanying drawings, in which—

Figure 1 shows the furnace conventionally in side elevation;

Fig. 2 is a transverse sectional view; and 70 Fig. 3 is an enlarged view showing a suitable form of chain conveyer.

The fire brick tunnel 1 is suitably supported by supports 2 and heated by series of burners 3. Supported on the staggered 75 bricks 4 is a hearth 5 having bearing plates 6 for the links 8 of the chain to which the cross bars 7 are secured. The endless chain passes over end rollers or sprockets 9 and 10, a suitable worm or other drive (not 80 shown) being provided for driving the sprocket 10. A supporting or guide rail 11 is provided for the endless belt on its return. Openings for the escape of products of combustion are indicated at 12. 85

In the operation of the apparatus the sheet metal ware is supported on the cross bars 7 or on projections therefrom, and is carried through the furnace and there heated in the manner above described. A sufficient length of the endless chain is provided 90 at the discharge end of the furnace so that the ware will be cooled before it is finally removed.

It will be evident that, in a furnace of the 95 character described, the temperature of the furnace and of different parts thereof, can be readily regulated.

The oxidation of the steel should not be carried too far and the oxid film produced 100 should not become too thick, otherwise it will not be entirely absorbed by the molten enamel during the enameling operation. The function of the layer or film of oxid, as I believe, is to provide a medium through 105 which the enamel is secured to the steel, so that the composition of the enamel changes progressively from pure enamel to enamel containing increasing quantities of iron oxid which is united to the underlying iron 110 by means of the iron oxid union. It appears to be essential for substantially all of the oxid film to be absorbed by the molten enamel, in order to obtain a proper union 115 of the enamel with the metal. Ground and polished cross sections of sheet steel which has been enameled after treatment in the manner above described, when examined microscopically in comparison with steel which has been pickled before enameling, 120 shows that the pickling does not, as is sometimes supposed, yield a surface which is rougher and promotes a better union of the enamel with the steel.

From the above description it will be seen 125 that the process of the present invention avoids the necessity for the usual cleaning and pickling treatment, that the burning off and removal of grease and other foreign matter from the steel ware can be effected 130

- by the same operation which results in the formation of an oxid coating, and that by the heating of the steel ware to the proper degree an oxid coating is formed to which 5 the enamel coating can be applied directly without any preliminary pickling operation. The optimum quantity of oxid that has been found desirable can be developed by the regulated heat treatment which is also sufficient 10 to completely volatilize or burn the oil present on the steel, and the steel, after such treatment, can be enameled directly without further preparation, and with the resulting production of an enamel comparable in quality to an enamel which has been applied to 15 pickled steel.

The enameling operation itself, to which the oxidized steel is subjected, may be the customary enameling operation to which 20 pickled steel is subjected, and this operation can be carried out in the usual way, *i. e.*, by applying the enamel to the oxidized surface, drying and firing.

I claim:—

- 25 1. The method of making enameled ware, which comprises subjecting sheet steel having an oil coating thereon to a regulated heating to remove the oil and form a blue oxid coating thereon, and subjecting the 30 resulting oxidized steel to an enameling operation, whereby preliminary treatment of the oiled surface for the removal of oil and subsequent pickling thereof prior to the enameling operation are avoided.
- 35 2. The method of producing enameled ware, which comprises subjecting sheet steel having an oil coating thereon to a drawing operation to produce ware of the desired shape, heating the ware to remove the oil 40 and produce a thin oxid coating thereon, applying the enameling composition to the oxidized surface, and firing the resulting ware, whereby preliminary treatment of the oiled surface for the removal of oil and subsequent 45 pickling thereof prior to the enameling operation are avoided.
3. The method of enameling steel ware having an oil coating thereon, which comprises subjecting the ware to a temperature 50 of about 700° C. for about 30 seconds to

remove the oil and produce an oxidized surface, and subjecting the resulting oxidized ware to an enameling operation, whereby preliminary treatment of the oiled surface for the removal of oil and subsequent pickling thereof prior to the enameling operation are avoided. 55

4. The method of enameling steel ware having an oil coating thereon, which comprises continuously passing the ware through 60 a furnace, heated to about 700° C., at such a rate that the ware will be subjected to such temperature for a period of about 30 seconds, and thereby removing the oil and producing a thin oxid coating, and subjecting 65 the resulting ware to an enameling operation, whereby preliminary treatment of the oiled surface for the removal of oil and subsequent pickling thereof prior to the enameling operation are avoided. 70

5. The method of preparing steel, iron and like metal surfaces for enameling which comprises subjecting such surfaces having an oil coating thereon to a regulated heating operation sufficient to remove the oil 75 and form a blue oxid coating thereon, whereby preliminary treatment of the oiled surface for the removal of oil and subsequent pickling thereof prior to the enameling operation are avoided. 80

6. The method of preparing sheet metal ware for enameling which comprises subjecting sheet metal having an oil coating thereon to a drawing operation to produce 85 ware of the desired shape and heating the drawn ware to remove the oil and produce a thin oxid coating thereon, whereby preliminary treatment of the oiled surface for the removal of oil and subsequent pickling thereof prior to the enameling operation are 90 avoided.

7. The method of preparing sheet metal ware for enameling which comprises subjecting the ware to a temperature of about 95 700° C. for about 30 seconds and thereby producing an oxidized surface adapted to receive the enameling composition.

In testimony whereof I affix my signature.

RAYMOND DENNY COOKE.